

## UNITED STATES PATENT OFFICE

LAWRENCE BRADSHAW AND HENRY V. DUNHAM, OF BAINBRIDGE, NEW YORK, AS-SIGNORS, BY MESNE ASSIGNMENTS, TO THE CASEIN MANUFACTURING COMPANY OF AMERICA, INC., OF NEW YORK, N. Y., A CORPORATION OF DELAWARE

PROCESS OF RETARDING THE SETTING OF CASEIN GLUE AND DRY GLUE BASE FOR USE IN SUCH PROCESSES

No Drawing.

Application filed April 2, 1926. Serial No. 99,423.

This invention has for its object improvements in casein waterproof glues or cements and in a novel "glue base" which when properly incorporated with water will produce 5 such an adhesive. It is well known that glues prepared from different commercial caseins exhibit wide variations in consistency when mixed with a given proportion of water and also differ greatly in their subsequent behavior, notably in the interval of time which 10 may elapse between the initial mixing with water and the point at which the glue "sets", i. e., becomes too thick to spread. Various methods have been proposed to control this 15 interval, generally termed the "life" of the glue, such as the addition of animal glue or salts of the alkali or alkaline earth metals. The use of animal glue for this purpose is uneconomical, since its natural strength, 20 which otherwise would contribute to the adhesiveness of the mixture, depreciates considerably under these conditions. The addition to casein glues of alkali metal phosphates, fluorides and other salts which by interaction 25 with lime liberate caustic alkalies is undesirable beyond a certain point; that is to say, any large excess over the amounts of produced caustic alkali sufficient to dissolve the casein and to impart a workable consistency 30 and ultimate water-resisting property to the glue, is to be avoided since the excess of free caustic alkali thus produced causes hydrolysis of the casein and consequent loss of strength.

35 We have now found that cottonseed meal or peanut meal added to casein waterproof glues have a marked effect in retarding the "setting" of the liquid glues, thereby extending the life of such glues. As an example, the 40 rates of change in the viscosity of a commercial casein glue (A) and of the same glue with 7% (B) and with 15% (C) respectively of pulverized cottonseed meal added are compared below. One part of each of the glue 45 bases was mixed with two parts of water at 60° F., producing a slight rise in temperature. The viscosities were determined at 70° F., in all cases. The values represent readings on the Stormer viscosimeter (provided with a 50 500 gram weight) at regular intervals after

mixing, the conditions of making and testing the three liquid glues A, B and C, being identical,

|        | 1 hr. | 3 hrs. | 5 hrs. | 7 hrs. | 9 hrs. | 11 hrs. | 13 hrs. |
|--------|-------|--------|--------|--------|--------|---------|---------|
| A----- | 26    | 9      | 2      | set    | -----  | -----   | -----   |
| B----- | 33    | 18     | 10     | 5      | 1      | -----   | not set |
| C----- | 27    | 21     | 15     | 8      | 5      | 3       | 1½      |

55

A further example shows the effect of adding 60 to another good casein glue (A') 7% of pulverized peanut meal, producing a mixed casein-peanut glue (P).

|         | 1 hr. | 3 hrs. | 5 hrs. | 7 hrs. | 8 hrs. |
|---------|-------|--------|--------|--------|--------|
| A'----- | 25    | -----  | -----  | -----  | -----  |
| P-----  | 24    | 10     | 6      | 9      | 2      |

65

We find that by substituting 50% of the casein 70 in a regular third good commercial casein glue (A'') by an equivalent amount of the pulverized peanut meal a glue (Q) is obtained which undergoes practically no change in viscosity over a long period, as shown in 75 the comparison below:

|          | 1 hr. | 3 hrs. | 5 hrs. | 7 hrs. | 8 hrs. |
|----------|-------|--------|--------|--------|--------|
| A''----- | 20    | -----  | -----  | -----  | -----  |
| Q-----   | 20    | 8      | 2½     | 22     | set 25 |

80

The "commercial casein glue" referred to above, was in each case, a pulverulent mixture consisting of casein, hydrated lime and alkali-metal salts capable of reacting with 85 the hydrated lime (when water is added) to produce caustic alkali and insoluble calcium salts. The proportions of said components were similar to the proportions given in the present application.

90

It will also be understood that by varying the proportions of the protein-rich meal added, the life of the glue can be controlled within wide limits. We prefer to use meal which has been ground to pass through a 120 95 mesh screen, although a coarser product of approximately 80 mesh has given good results in casein waterproof glues. With the finer meal a smoother glue is obtained.

In carrying out the invention the casein 100

(that is, casein from milk) is mixed dry, with an appropriate amount of the vegetable meal, and to this mixture is added an alkaline earth metal hydroxide and preferably also one or more alkali metal salts capable of dissolving the proteins. The following examples of mixtures which have given satisfactory results when applied to joints and laminated woods will serve to illustrate more particularly the character of the invention, but we do not desire to be limited to the particular compounds or proportions herein set forth. (The parts are by weight).

*Example 1.*—Casein 60 parts; cottonseed meal 120 mesh, 10 parts; hydrated lime 15 parts; sodium fluoride 5 parts, sodium carbonate 5 parts; tri-sodium phosphate 3 parts, (98 parts in all).

*Example 2.*—Casein 33 parts, cottonseed meal 33 parts, hydrated lime 20 parts, sodium fluoride 6 parts, sodium carbonate 8 parts, (100 parts in all).

*Example 3.*—Casein 50 parts, cottonseed meal 20 parts, hydrated lime 15 parts, magnesium oxide 5 parts, sodium fluoride 7 parts, tri-sodium phosphate 3 parts, (100 parts in all).

*Example 4.*—Casein 40 parts, peanut meal 30 parts, hydrated lime 18 parts, sodium fluoride 5 parts, sodium carbonate 5 parts, sodium arsenate 1 part, (99 parts in all).

*Example 5.*—Casein 50 parts, peanut meal 22 parts, hydrated lime 18 parts, sodium carbonate 10 parts, (100 parts in all).

*Example 6.*—Casein 54 parts, peanut meal 30 parts, hydrated lime 16 parts. One part of the dry mixture is to be incorporated with about 3 parts of cold water.

These examples indicate the dry materials which are mixed together to form the glue base. The dry mixture is incorporated with water (at or just before the time of use), by the methods well known to users of casein glues. We prefer to use from 2 to 2½ parts of cold water to 1 part of the dry base. The water is put into a kettle provided with an efficient stirring device; the dry glue base (e. g. one of the above formulas) is added slowly and mixed thoroughly for about 20 minutes and the glue is then ready for use.

The term "casein" is used herein in its usual significance, to denote certain coagulable phosphorus-containing protein matter as found in milk and skim milk.

55 The cottonseed meal preferably used (as referred to in Examples 1, 2 and 3) is the product obtained by grinding the cake left after pressing cottonseed (after removal of the major part of the hulls, and adhering fine 60 lint if desired) for the purpose of expressing the oil; it usually still contains some oil (perhaps 7-8%). It will be understood that the further removal of oil by solvent treatment of the press cake, or the direct extraction of the oil from the seed with suitable solvents

(e. g. after decorticating and comminuting) are not precluded. It will also be understood that the use of the oil-extracted or partially extracted seed, containing substantially all the hull material is likewise not precluded. The term "cottonseed meals" as used herein, is intended to cover such products as are referred to in this paragraph.

In the above specification reference has been made mainly to cottonseed meal but we 75 wish it understood that peanut meal can be used in a precisely similar manner, and is accordingly considered as an equivalent, and the term protein-rich "seed meal" as used in the claims is intended to cover cotton seed 80 meal and peanut meal.

The term "alkaline earth oxide" as used in the appended claims is intended to embrace this material in the anhydrous or hydrated states, and also the corresponding oxide and hydroxide of magnesium. The term "salt" is intended to be used in the generic sense to include the singular or plural forms, i. e. one salt or several salts. The statement in any claim that the material will pass a screen 85 of particular mesh does not mean that the material (or some part thereof) will not pass through a finer screen. Alkaline substances, e. g. sodium carbonate, borax, etc. are capable (with water) of dissolving casein and 90 meal proteids.

We claim:—

1. A new dry base for use in making an adhesive material comprising casein as a substantial ingredient together with a substantial amount of a protein-rich seed meal, incorporated with an alkaline earth oxide and a water-soluble alkali metal salt which reacts alkaline to litmus, and which salt is capable of reacting in the presence of water, with such alkaline earth oxide, which base is adapted upon being subsequently mixed with sufficient water, to produce a fluid adhesive of spreadable consistency.

2. A new dry base for use in making an adhesive composition containing casein as a major ingredient together with a relatively smaller but substantial amount of cotton seed meal from which most of the oil has been separated, and a water-soluble alkali metal salt which salt reacts alkaline to litmus, which base is adapted upon being subsequently mixed with sufficient water to produce a fluid adhesive of spreadable consistency.

3. A new dry base for the manufacture of glue and adhesive compositions, such base comprising casein, a lesser but substantial amount of protein-rich seed meal ground to pass an 80 to 120 mesh screen, an alkaline earth oxide in amount sufficient to maintain the mixture alkaline, and a substantial amount of a water-soluble alkali metal salt which in aqueous solution will react with the said alkaline earth oxide to produce a solvent for the casein and for the protein of said 120 125 130

- protein-rich seed meal, which base, upon being subsequently mixed with cold water will form a fluid adhesive. 102
4. A new dry base for the manufacture of glue and adhesive compositions, such base comprising casein and a protein-rich seed meal from which a large part of the hull substance has been removed, ground to pass an 80 to 120 mesh screen, such casein and seed meal both being present in substantial amount, an alkaline earth oxide, in amount sufficient to maintain the mixture alkaline and a substantial amount of a water-soluble alkali metal salt which in aqueous solution will react with the said alkaline earth oxide to produce a solvent for the casein and for the protein of said protein-rich seed meal, which base, upon being subsequently mixed with cold water will form a fluid adhesive. 150
5. A new dry base for the manufacture of glue and adhesive compositions, such base comprising casein, a lesser but substantial amount of protein-rich seed meal from which a substantial part at least of the oil has been removed, ground to pass an 80 to 120 mesh screen, an alkaline earth oxide in amount sufficient to maintain the mixture alkaline, and a substantial amount of a water-soluble alkali metal salt which in aqueous solution will react with the said alkaline earth oxide to produce a solvent for the protein, which base, upon being subsequently mixed with cold water will form a fluid adhesive. 200
6. A new dry base for the manufacture of glues and adhesive compositions, such base comprising casein and a protein-rich seed meal from which a substantial part at least of the oil has been removed, the major part at least of which meal is fine enough to pass an 80 to 100 mesh screen, and an alkaline earth oxide in amount sufficient to maintain the mixture alkaline when water is added, both the casein and the meal being present in substantial amounts, and the casein and meal together constituting the major part of said base, which base, upon being subsequently mixed with cold water will form a fluid adhesive. 250
7. A new dry base for the manufacture of glues and adhesive compositions, such base comprising casein, a lesser amount of fine protein-rich seed meal, and an alkaline earth oxide in amount sufficient to maintain the mixture alkaline when water is added, the amount of such meal being sufficient to substantially lengthen the life of the adhesive prepared from said base, as compared with a casein glue without such seed meal. 300
8. A new dry base for use in making an adhesive material comprising casein as a substantial ingredient, together with a substantial amount of a protein-rich seed meal, incorporated with an alkaline earth oxide and a water-soluble alkali metal salt, which salt is capable of reacting, in the presence of water, with such alkaline earth oxide, which base, upon being subsequently mixed with sufficient water, will produce an adhesive of fluid spreadable consistency. 350
9. A novel material in the glue art, the same being an intimate dry mixture comprising casein and a protein-rich seed meal, the former being in excess of the latter. 400
10. A novel material in the glue art, the same being an intimate dry mixture comprising casein and a protein-rich seed meal, the amount of casein being substantially greater than the amount of protein contained in the seed meal. 450
11. A dry glue base containing about equal parts of casein and of a dry protein-rich seed meal, together with smaller amounts of an alkaline earth metal oxide and of alkaline-reacting sodium salt, the latter being in amount sufficient, by reaction with the said alkaline earth metal oxide, to form a solvent for the casein and meal proteids present. 500
12. A process for producing a glue of comparatively long working life from a glue base including casein, a water-soluble alkali metal salt which is alkaline to litmus, and an alkaline earth metal oxide, which process comprises incorporating a protein-rich seed meal in such glue base, and thereafter mixing this new glue base with water, the proportion of the protein-rich seed meal used being sufficient to retard the setting of the glue produced by said admixture with water. 550
- In testimony whereof we affix our signatures. 600
- LAWRENCE BRADSHAW.  
HENRY V. DUNHAM. 650
- 105
- 110
- 115
- 120
- 125
- 130